

Patented Oct. 23, 1928.

1,688,799

# UNITED STATES PATENT OFFICE.

ALBERT BODMER, OF WATTWIL, SWITZERLAND, ASSIGNOR TO HEBERLEIN & CO., A. G.,  
OF WATTWIL, SWITZERLAND, A CORPORATION OF SWITZERLAND.

## FABRIC MAKING.

No Drawing. Original application filed November 27, 1926, Serial No. 151,258, and in Germany December 5, 1925. Divided and this application filed July 14, 1928. Serial No. 292,922.

My invention relates to improvements in fabric making, and more particularly to fabrics with pattern effects. Dense patternings on a relatively light weight ground or foundation fabric have heretofore been produced by providing a fabric having some threads therein which before weaving have been treated with a carbonizing agent, so-called, and after weaving protecting portions of these threads with a resist according to a predetermined pattern and destroying the remaining portions of the treated threads with the aid of heat, leaving the other portions thereof still woven in the fabric and forming a pattern effect therein. Such a method is disclosed in United States Patent No. 1,425,520, granted August 15, 1922.

According to the method of said prior patent, however, it has been found that as a practical commercial matter difficulties arise in practice resulting in a loss of yarn unless great care is taken. Under that process the yarns were dried at low temperature in an endeavor to reduce loss, but even so some loss occurred. This is due to the fact that the yarns when treated with sulphuric acid are partially destroyed while drying. Waste has also been experienced in moisture getting to the yarns in transmission from the yarn or spinning mill to the weaving mill. The old process also involved the necessity of using a beating machine or the like after the carbonization had taken place to remove the carbonized fibres.

According to the present invention more or less similar pattern effects are obtained without such carbonization of the threads. The new process is simpler, much more reliable, and avoids the losses under the old process. This application is a division of my copending application Serial No. 151,258, filed November 27, 1926, for fabric making.

In carrying out the invention in a preferred form thereof, I produce a fabric having a foundation or ground work of any suitable threads, but preferably of cotton or other threads of vegetable or cellulosic matter (including artificial silk), said ground work having interwoven therein threads of nitrated vegetable or cellulosic material such as nitrated cotton threads. These nitrated threads may be in the warp or in the woof or may run in both directions with the

unnitrated threads which form the foundation. The nitrated threads may alternate singly or in numbers with the untreated threads of the foundation or the nitrated threads may be twisted with the unnitrated foundation threads or some of them. 55

After such a fabric has been produced with nitrated threads associated therewith, I preferably cause an alkali such as a solution of caustic soda, to act on the nitrated threads in various spots or places according to a predetermined design or pattern, and where the alkali is thus brought into contact with the nitrated threads it dissolves or decomposes the same, so that the portions of the nitrated threads so attacked are destroyed and may be easily removed in any suitable manner, such as by washing. This leaves only the ground work or foundation at these places so that the remaining portions of the fabric containing the unattacked nitrated threads presents a raised pattern effect on the foundation. The action of the alkali on the nitrated threads may be accelerated by dry heat or steaming during the operation. 60

The localized action of the alkali, on the nitrated threads may be effected preferably by printing a relatively thick alkali solution on the fabric according to the predetermined design. Or if desired a resist that will immunize the threads against the alkali may be printed on the fabric according to a predetermined design and then the fabric passed through an alkali solution. In this way only the portions of the nitrated threads not protected by the resist are decomposed or destroyed. In my said parent application I have claimed the invention generically and have also made specific claims to the first of the two ways of carrying out the invention above described, whereas in this application I aim to cover the second of the two foregoing methods of carrying out the invention. 65

Also substantially the same result may be obtained but in a less satisfactory manner, by printing a denitrating agent on the fabric according to a predetermined design thereby rendering portions of the nitrated threads inert to the alkali, and thereafter passing the fabric through the alkali solution whereby only the portions of nitrated threads which have not been denitrated are destroyed. Similarly but also in a less satisfactory manner a resist to the 70

75

80

85

90

95

100

105

denitrating agent may be printed on the fabric according to a predetermined design and then the fabric passed through the denitrating agent to denitrate the unprotected portions of the nitrated threads, after which the resist may be removed and the fabric subjected to the alkali solution to destroy the portions of the nitrated threads which remain nitrated, so that the undecomposed or unattacked portions of the nitrated threads terminate at various points or along various lines in the fabric and thereby produce a pleasing pattern effect in a simple manner. That is, in the places where no denitration has taken place the nitrated threads are decomposed and removed.

The nitration of the cellulosic or vegetable threads may be effected in any well known or suitable manner, for example, with a suitable mixture of sulphuric and nitric acids. It is generally not necessary to nitrate very strongly, but according to the kind of threads employed and the method of carrying out the alkaline or decomposing treatment, the degree of nitration may vary within wide limits. But it will be understood, of course, that in no case is the nitration carried to the extent where it will materially reduce the tensile strength of the threads or yarn so that they would not have the necessary tensile strength for weaving. The degree of nitration is therefore different from that practised in the nitration of fibres in other cases where nitration is carried on for other purposes without the requirement of maintaining the necessary degree of tensile strength of the fibres for weaving. Even by the use of nitric acid alone (without the use of sulphuric acid) it is often possible to obtain a nitration that is sufficient for the purposes in question.

After the removal of the portions of the nitrated threads which have been destroyed by the alkaline treatment or by dissolving action, if the remaining portions of the nitrated threads have not already been denitrated as above explained, I preferably then denitrate the same. This is especially expedient in the case of relatively highly nitrated products and puts the completed fabric in a condition such that it will not thereafter be subject to attack by alkalies as would be the case if threads were left therein in a nitrated condition; and the denitration also improves the dyeing qualities of the goods.

The invention may be applied to fabrics of many different kinds, such for example as to fabrics composed of vegetable threads only, or of mixtures of vegetable, animal and artificial threads, or of any two of them, or to artificial silks and to embroidery materials. The nitrated threads may be produced from any suitable vegetable or cellulosic fibres, such for example as from ordi-

nary vegetable fibre threads or artificial silk threads.

Thus while I have described my improvements in detail and with respect to certain preferred forms, I do not desire to be limited to such details or forms since, as will be understood by those skilled in the art after understanding my invention, many changes and modifications may be made and the invention embodied in widely different forms without departing from the spirit and scope thereof in its broader aspects, and I desire to cover all modifications, forms and embodiments coming within the language or scope of any one or more of the appended claims.

Having thus described my invention, what I claim as new and desire to secure by Letters Patent, is:

1. Method of producing fabrics with pattern effects which consists in taking for treatment a fabric containing unnitrated threads and nitrated cellulosic threads, applying to the fabric according to a predetermined design a reserve which is resistant to the action of a reagent which will decompose the nitrated threads with which it comes into contact and subjecting unreserved portions of the fabric to said reagent to decompose the nitrated threads in such last portions.

2. Method of producing fabrics with pattern effects which consists in taking for treatment a fabric containing unnitrated threads and nitrated cellulosic threads, applying to the fabric according to a predetermined design a reserve which is resistant to the action of an alkali and subjecting unreserved portions of the fabric to said alkali to decompose the nitrated threads in such last portions.

3. Method of producing fabrics with pattern effects which consists in taking for treatment a fabric containing unnitrated threads and nitrated cellulosic threads, applying to the fabric according to a predetermined design a reserve which is resistant to the action of caustic soda, subjecting the unreserved portions of the fabric to caustic soda and heat to decompose the nitrated threads in such last portions, and removing the decomposed threads.

4. Method of producing fabrics with pattern effects which consists in producing a fabric with unnitrated threads and nitrated cellulosic threads therein, applying to the fabric according to a predetermined design a reserve which is resistant to the action of a reagent which will decompose the nitrated threads with which it comes into contact, and subjecting the unreserved portions of the fabric to said reagent to decompose the nitrated threads in said last portions.

5. Method of producing fabrics with pattern effects which consists in producing a fabric with unnitrated threads and nitrated

cellulosic threads therein, applying to the fabric according to a predetermined design a reserve which is resistant to the action of a reagent which will decompose the nitrated threads with which it comes into contact, subjecting the unreserved portions of the fabric to said reagent to decompose the nitrated threads in such last portions, denitrating the remainder of the nitrated threads

10 and removing the decomposed threads.

6. Method of producing fabrics with pattern effects which consists in producing a fabric with unnitrated threads and nitrated cellulosic threads therein, applying to the

15 fabric according to predetermined design a reserve which is resistant to the action of an alkali and subjecting the unreserved portions

of the fabric to said alkali to decompose the nitrated threads in such last portions.

7. Method of producing fabrics with pattern effects which consists in producing a fabric with unnitrated threads and nitrated cellulosic threads therein, applying to the fabric according to a predetermined design a reserve which is resistant to the action of 20 caustic soda, subjecting the unreserved portions of the fabric to caustic soda and heat to decompose the nitrated threads in such last portions, removing the decomposed threads and denitrating the reserved nitrated 25 threads.

In testimony whereof I have signed my name to this specification.

ALBERT BODMER.